

## [54] METHOD FOR REFINING OF STEEL MELTS

[75] Inventor: **Bertil G. Tivelius, Viken, Sweden**[73] Assignee: **Scandinavian Lancers Aktiebolag, Hoganas, Sweden**[21] Appl. No.: **367,796**[22] Filed: **Apr. 12, 1982**[51] Int. Cl.<sup>3</sup> ..... **C21C 7/10**[52] U.S. Cl. ..... **75/49; 75/53; 266/158**[58] Field of Search ..... **75/49, 53; 266/158**

## [56] References Cited

## U.S. PATENT DOCUMENTS

3,501,290 3/1970 Finkl ..... **75/49**

Primary Examiner—P. D. Rosenberg

Attorney, Agent, or Firm—Murray and Whisenhunt

## [57] ABSTRACT

A method for refining of steel melts for production of steel, especially stainless steel, with extremely low oxygen content is characterized in that a powdered non-oxidic earth alkali metal compound or alloy is injected

by means of a non-oxidizing carrier gas, preferably an inert gas, into a well de-oxidized steel melt which is covered by a basic reduced slag in a metallurgical ladle, whereby at least a significant amount of the earth alkali metal is oxidized by the oxygen dissolved in the melt to form small particles of earth alkali metal oxide, of which some are separated out to the slag cover while the remaining portion of the earth alkali metals stays behind in the melt in elementary form or combined in the form of particulate earth alkali metal oxide in colloidal solution, and that then powdered earth alkali metal oxide is injected, whereby there latter, larger oxide particles function as nucleus forming agents for the continued reaction between earth alkali metals dissolved in the melt and oxygen, and also for separation to the slag cover of smaller inclusions already existing in the melt. There is also provided an equipment for carrying out the method comprising a hood arranged above the ladle and designed so as to prevent air from entering into the space between the hood and the surface of the steel melt.

11 Claims, 1 Drawing Figure





## METHOD FOR REFINING OF STEEL MELTS

## TECHNICAL FIELD

The invention relates to a method for refining steel melts for the production of steel, especially stainless steel, with extremely low oxygen content. More precisely the invention relates to an injection metallurgical method for reducing the oxygen content in steel melts to extremely low levels. The invention also relates to equipment for carrying out the method.

## BACKGROUND TO THE INVENTION

In the metallurgy of steel, injection technique is playing an increasingly important role for the development of continuously improved steel qualities. By injecting fine particle size calcium and/or magnesium compounds or alloys it has thus for example been possible to reduce the total content of sulphur in steel melts to extremely low values. By selecting suitable injection products it has also been possible to transform residual sulphides so that these become as harmless as possible. For example U.S. Pat. No. 4,261,735 describes a method in accordance with which lime, CaO, is initially injected and then when the majority of the sulphur has been removed, injection is continued with calcium-silicon, SiCa, calcium carbide, CaC<sub>2</sub>, and/or calcium cyanamide, CaCN<sub>2</sub>.

In modern metallurgy it has also been possible to reduce the content of oxidic inclusions to very low levels. Traditionally the majority of the oxygen in steel melts is removed by de-oxidation using a suitable de-oxidising agent, usually aluminium, silicon or manganese. To reduce the oxygen content to values lower than those which can be achieved using aluminium, silicon and manganese it is necessary however to employ more effective oxidising agents. The substances which can be mainly considered are earth alkali metals in the elementary or non-oxidic-combined form. In actual practise this usually signifies calcium, although also magnesium can be employed as an alternative to calcium. For example calcium can be added in metallic form, as a wire encapsulated in a plate metal casing. Calcium can also be added as calcium-silicon, although the maximum permissible silicon content in the steel imposes a limit on how much calcium-silicon can be added. Furthermore in actual practice it has proved difficult to reduce the oxygen content in this way. The same applies to the injection of calcium carbide CaC<sub>2</sub>, which in addition signifies that the melt is carburised and this is not acceptable in many cases, particularly not when producing low carbon content stainless steel or other steels with very low carbon content.

In the search for increasingly improved grades of steel requirements have now been imposed for extremely low oxygen contents, meaning not more than 5 ppm and preferably not more than 2 ppm dissolved oxygen in the liquid steel after the injection treatment. The aim of these extremely low oxygen contents is to reduce the total quantity of oxidic inclusions in the finished steel. By reducing the content of oxidic inclusions, mainly inclusions of the Al<sub>2</sub>O<sub>3</sub> type, it is thus possible to considerably reduce the number of rupture initiators. Furthermore the polishability of the steel can be improved which in many cases is a desirable property for stainless steel and tool steels. The low oxygen content also has advantages from the viewpoint of the metallurgical process, because a low content of oxidic

inclusions improves the viscosity of the steel and reduces the risk of blockages during the casting of the steel. Furthermore a low oxygen content is a pre-requisite if extremely low sulphur contents are also to be achieved, because the oxygen activity in the steel melt determines the course of desulphurisation.

The extremely low oxygen contents required in accordance with the invention, i.e. not more than 5 ppm and preferably not more than 2 ppm, could not however be achieved at reasonable cost with high reproducibility using methods known hitherto unless at the same time quality requirements other than the low oxygen content were abandoned.

## DISCLOSURE OF THE INVENTION

The aim of the invention is to provide a method, with high economy and good reproducibility, of refining steel melts for the production of steel, particularly stainless steel with extremely low oxygen content, i.e. not more than 5 ppm and preferably not more than 2 ppm in the molten steel. In accordance with the invention different earth alkali metal compounds or alloys, preferably calcium compounds or alloys, are injected in one or several sequences. Each such sequence comprises the injection of calcium-silicon, SiCa, in the form of powder by means of a non-oxidising carrier gas, whereby silicon is dissolved into the melt whilst at least a significant portion of the calcium is oxidised by the oxygen to form small particles of calcium oxide, CaO, of which some are separated to the slag cover whilst the remainder of the calcium stays behind in the melt in elementary form or combined in the form of particulate calcium oxide in colloidal solution. Preferably the amount of SiCa injected is such that by this means the content of dissolved oxygen in the melt is reduced to at least half. Then powdered calcium oxide, CaO alone or, preferably, together with fluorspar, CaF<sub>2</sub>, is injected whereby these latter larger CaO particles function as nucleus forming agents for the continued reaction between calcium and oxygen dissolved in the melt, and also for separating smaller inclusions already present in the melt to the slag covering.

The method described of injecting SiCa followed by injection of CaO can be repeated once or several times so as to further reduce the oxygen content in the melt during each sequence.

Simultaneous with the injection of CaO it is also possible to add other calcium compounds such as CaF<sub>2</sub>. A conceivable CaF<sub>2</sub> content in the combined CaO and CaF<sub>2</sub> addition is 10-30 weight-%, suitably about 20%. It is also possible to envisage the addition of other non-oxidic-bound calcium compounds, e.g. calcium carbide CaC<sub>2</sub> and/or calcium-cyanamide, CaCN<sub>2</sub>, during the injection of calcium-silicon, SiCa. Instead of calcium compounds in the sequence described above it is also possible to envisage the use of magnesium compounds of the corresponding type.

It should also be mentioned that prior to the injection of the said compounds the steel melt must be de-oxidised and covered by a basic, reduced slag in a metallurgical ladle. Conventional de-oxidising agents such as aluminium, silicon or manganese can be used for de-oxidation, and known reduction agents such as aluminium and silicon can also be employed for reduction. For example it can be appropriate to use silicon in the form of calcium-silicon, SiCa, whereby the simultaneous

admixture of SiCa can represent the first stage of the sequence of injections in accordance with the invention.

To permit rapid change overs from one substance to another during the sequential injection of the said compounds it may be appropriate to make use of for example the method employing two or more series-connected powder emitters as described in U.S. Pat. No. 3,998,625.

It should also be mentioned that apart from oxygen reduction very efficient sulphur refining is also achieved, in that some of the calcium in the injected calcium-silicon combines with the sulphur dissolved in the melt, after which the calcium sulphide formed collects in the slag cover. Also the injected calcium oxide, like the calcium oxide formed in situ in the melt, can contribute in a corresponding manner towards reducing the sulphur content, especially if the oxygen in the melt is approaching extremely low values. Actually an injection of calcium oxide undertaken in accordance with a conventional method should result in a reduced sulphur content, whilst on the other hand the oxygen content would not be further reduced. In the case of the procedure in accordance with the invention however as a result of the sequence selected at the same time a continued reduction of oxygen is obtained during the injection of CaO.

In the method use is made of a wholly or partially basiclined ladle. The ladle can for example be lined with dolomite. The equipment in accordance with the invention also comprises a hood which during refining is placed above the ladle. The hood contains firstly a heat shield which essentially covers the ladle, although a gap is left between the heat shield and the upper edge of the ladle, also a screen which extends across and below the said gap so that a circumferential opening is formed between the screen and the ladle below the said gap. Furthermore at least one exhaust pipe is provided to communicate with the space underneath the said screen to suck out exhaust gases which pass from the ladle chamber out into the said space through the said gap, and also air which flows in from the ambient atmosphere through the opening between the screen and the outside of the ladle. Furthermore at least one aperture is provided in the hood for at least one lance which can be lowered into the space underneath the heat shield and/or into the melt in the ladle.

In accordance with a preferred embodiment the screen forms an all-closing roof over the heat shield, where the said aperture or apertures also extend through the screen over the heat shield, and where the entire space between the screen and the heat shield is so arranged as to be ventilated by sucking out through the said exhaust pipe. The equipment can be designed for two lances, namely an injection lance and a gas purging lance, arranged so that they can be introduced simultaneously into the ladle chamber under the heat shield through two apertures in the hood. One lance aperture is appropriately arranged centrally whilst the other aperture is displaced to the side.

#### DESCRIPTION OF THE PREFERRED EMBODIMENT

A detailed description with reference to the appended drawings which show a section through a ladle with a hood in accordance with the invention will now be given of a preferred embodiment of the equipment in accordance with the invention. The ladle has been generally designated as 1, a steel melt by 2 and a slag cover

by 3. Above the ladle 1 a hood generally designated as 4 is provided. The hood 4 can rest, with the support provided for the purpose, on the upper edge of the ladle 1 or be kept in place by means of an arm 5 which can be raised, lowered and pivoted. As a third alternative the hood can be suspended in chains beneath a platform. The hood 4 consists of a heat shield 6 with ceramic lining which faces the slag cover 3. A gap between the heat shield 6 and the upper edge 8 of the ladle is designated as 9.

Above the heat shield 6 a screen 10 is provided having a central section 11 which is joined to the upper steel casing 12 of the heat shield by a circular intermediate wall 13 with apertures 14. From the central section 11 the screen 10 extends, by way of a peripheral section 15 beyond the edge 8 of the ladle 1 and down past the gap 9 to a level underneath the edge 8. The opening between the projecting portion of screen 10 and the outside of ladle 1 is designated as 16, whilst the space between the shield 6 and the screen 10 is designated as 17. An exhaust pipe 18 is connected to the space 17.

The heat shield 6 and the screen 10 are provided with two pairs of concentric apertures 19, 20 and 21, 22. The two first mentioned apertures 19, 20 are arranged centrally and are designed for an injection lance 23 with a lance manipulator 24, whilst the two other apertures 21, 22 are arranged at the side thereof and designed for a gas purging lance 25. Both lances 23 and 25 can be brought down into and up from the melt 2. The gas purging lance 25 can also be introduced into the ladle chamber underneath the heat shield 6 without being introduced into the melt 2.

During operation, whether the gas purging lance 25 is immersed in the melt or not, inert gas is supplied under pressure above atmospheric pressure to the ladle chamber 26 between the heat shield 6 and the slag covering 3. The inert gas is supplied to the said space through the injection lance 23 and/or through the gas purging lance 25. The gases flow out through the gap 9 to the space 17 which is kept under vacuum in comparison with the ambient atmosphere by means of exhaustion through pipeline 18. At the same time a certain amount of air flows in through the opening 16, which air is mixed with the gases in the space 17 and is withdrawn together with the gases through pipeline 18, thus preventing any noticeable quantities of air flowing into the ladle chamber 26. By keeping the space 17 under vacuum, (under-pressure) with reference to the ambient atmosphere, it is also ensured that no considerable quantities of air flow into the ladle chamber 26 through the lance apertures 19-22.

I claim:

1. A method for refining steel melts to produce steel of reduced oxygen content, comprising providing a deoxidized steel melt covered by a basic reduced slag in a metallurgic ladle, and injecting at least one member selected from the group consisting of powdered non-oxidic earth alkali metal compound and alloys of said earth alkali metal by means of a non-oxidizing carrier gas into said deoxidized steel melt to oxidize at least a significant amount of the earth alkali metal by oxygen dissolved in the melt to form small particles of earth alkali metal oxide, with a portion of said earth alkali metal separating out to the slag while the remaining portion remains in the melt in a form selected from the group consisting of the elementary form and the particulate earth alkali metal oxide in colloidal solution form, and thereafter injecting powdered earth alkali metal

oxide into the steel melt to function as nucleus forming agents for the continued reaction between oxygen and earth alkali metal dissolved in the melt, and to separate to the slag smaller inclusions in the melt.

2. Method of claim 1, wherein the steel which is produced is a stainless steel.

3. Method of claim 1, wherein said non-oxidizing carrier gas is an inert gas.

4. Method as claimed in claim 1, wherein a significant quantity of fluorospar,  $\text{CaF}_2$ , is supplied to the steel melt together with said earth alkali metal oxide.

5. Method of claim 4, wherein the amount of fluorospar is between 10 and 30 weight percent of the total of 15 said earth alkali metal oxide plus fluorospar.

6. Method of claim 5, wherein said amount is about 30 weight percent fluorospar.

7. Method as claimed in any one of claims 1, 2, 3 or 4, 20 wherein the amount of said member injected in said

melt is at least sufficient to reduce the dissolved oxygen content of the melt to a half.

8. Method of any one of claims 1, 2, 3 or 4, wherein the injection of said member followed by injection of 5 said earth alkali metal oxide is repeated at least once so as to further reduce the oxygen content during each injection sequence.

9. Method of any one of claims 1, 2, 3 or 4, wherein said member is selected from the group consisting of 10 calcium-silicon, calcium carbide, and mixtures thereof, and said earth alkali metal oxide is calcium oxide.

10. Method of claim 9, wherein said member is calcium-silicon.

11. Method of any one of claims 1, 2, 3 or 4, wherein during said injection sequence the ladle is covered by a hood, and the area above the surface of the steel melt is filled by a non-oxidizing gas under overpressure in comparison with ambient atmosphere to prevent air from entering into the ladle area above said steel melt to effectively prevent reoxidation of the melt.

\* \* \* \* \*

25

30

35

40

45

50

55

60

65